

S. Darling.  
Straight-Edge.

Nº 73082

Patented Jan. 7, 1868.



Inventor:

Samuel Darling  
by Crosby Hall and Alfred  
Big Attorneys

Witnesses.

Newton Jones

S. Darling.  
Straight-Edge.

Nº 73082

Patented Jan. 7, 1868.

Fig. 3.



Fig. 4.



Fig. 5.



Witnesses.

Newton Towner

Inventor:

Samuel Darling  
by Crosby, Halested & Gould  
his Attorneys

# United States Patent Office.

SAMUEL DARLING, OF BANGOR, MAINE.

*Letters Patent No. 73,082, dated January 7, 1868.*

## IMPROVEMENT IN STRAIGHT-EDGES.

The Schedule referred to in these Letters Patent and making part of the same.

TO ALL WHOM IT MAY CONCERN:

Be it known that I, SAMUEL DARLING, of Bangor, in the county of Penobscot, and State of Maine, have invented certain Improvements in Straight-Edges; and I do hereby declare that the following, taken in connection with the drawings which accompany and form part of this specification, is a description of my invention sufficient to enable those skilled in the art to practise it.

The object of my invention is the production of a tool or implement, usually designated by machinists and artisans, a "straight-edge," which shall have greater durability and toughness, less liability to be fractured or bruised, and greater hardness at its edges than any heretofore known or used, and which shall, also, when made with a graduated scale thereon, to serve as a rule or measure, insure great accuracy and reliability in such scale, as well throughout its entire length, as also for each of its aliquot parts into which it may be divided and subdivided.

Straight-edges, as heretofore made, have been usually formed from steel or other metal which is of homogeneous character and hardness throughout. If this be a soft metal, the implement, from its frequent handling and being left about, and thrown down upon the benches amongst other metal articles or tools, is constantly liable to become indented or nicked at its edges and corners, until soon it becomes so injured and untrue as to be valueless.

If, in order to avoid these liabilities to damage, it be made of harder material, such as hardened plate-steel, and of homogeneous character and texture throughout, it is in such case, by reason of its brittle nature, in constant danger of being fractured or broken, and in either case rendered useless.

Such tools being frequently broken, and even from slight blows and shocks, to which, in a machine-shop, they are constantly subject, it is, even as a mere matter of economy only, highly important to provide a straight-edge, which, whilst possessing at its edges the requisite degree of hardness for all purposes for which it may be used, shall at the same time have its mass or body, except at or near the edges, of such character or texture as to be but little, if any, liable to fracture, indentation, or abrasion, and thus serve to preserve the entire instrument for a long period in efficient working condition. Such a straight-edge forms the subject of my present invention.

Figure 1, of the accompanying sheet of drawings, represents my improved straight-edge, with a scale graduated thereon in the manner hereinafter described, and after the same has been polished, ready for use; and

Figure 2 represents the same, after the edges thereof have been hardened, but before the surface has been ground or polished.

Figures 3, 4, and 5, represent modifications and cross-sections of the same.

In making my improved straight-edge, I take a piece of steel plate, of the length, breadth, and thickness desired, and heat it to a proper temperature and dip it into water; but before so heating and dipping it, I confine the plate between two blocks of iron, and in order to limit the effects of the hardening-process to the edges only, I allow the edges so to be hardened, to project beyond the said confining-blocks. The two blocks and the interposed plate are then heated together, and while the blocks serve to prevent the contact of the water with the heated plate, except at its projecting edges, they also serve to keep up the temperature of the centre of the plate, so that it does not cool so rapidly as to become brittle. The same result may be attained by tempering or hardening the edges by pressure between surfaces of cold iron, leaving the centre unchanged. After being thus tempered, the plate, if warped, as it is apt to be by the tempering-process, is rendered true by hammering, and its edges ground straight and smooth, the opposite ones being made parallel.

A straight-edge cannot long remain accurate when its edges are soft, and easily worn or indented; but if the whole plate be hardened alike, besides being in such case brittle, it becomes very much warped and twisted, and being in this state very refractory, these warps and twists do not admit of being hammered out. By my improvement, however, the edges alone being hardened, the whole plate admits of being hammered on the sides to remove the warps and twists incident to the hardening-process.

My manner of obtaining the correct graduation of the hardened straight-edge is as follows: I find by experiment that the edges will, in the hardening-process, expand about one twenty-fifth ( $\frac{1}{25}$ ) of an inch to the foot. I therefore cut and graduate them, before hardening the edges accurately, to one twenty-fifth of an inch to the foot short of the standard measure.

In preparing and hardening the edges of a number of plates, it is found, however, that they will not all expand alike. I, however, make them all alike at first, and afterwards bring or reduce each one to the exact standard, by drawing the temper. In order to do this, they must all be made long enough to permit this reduction or shortening. To effect this, I use a hot bath of oil or tallow, and the more the straight-edge needs to be shortened, the hotter the bath must be. The degree of heat necessary for this purpose must be learned by practice. If one edge be longer than the other, then that edge alone must be put into the bath, until it be brought down to the true standard of the other; and the edge not so being heated may be clamped with metal when necessary to keep it from heating.

It is apparent from the above that either or both edges, as the case may require, and to a greater or less extent, may be contracted, until the precise desired standard be obtained.

It is often necessary or desirable to have a straight-edge of great length, even to the extent of twenty feet or thereabouts. To make such a one in a single piece would be very difficult and inconvenient, if not impracticable. I therefore make it in sections, of, say, four straight-edges, each five feet long, and each with hardened edges, made as above described; and after first making in each two or more slots, in a direction transverse of their lengths, for the reception of screws, I affix these sections, placed end to end, by means of screws, to a wide, well-seasoned board, and secure them in position, so that their hardened edges shall be in a continuous straight line; and in order to true these edges before finally securing them in position, I make use of another straight-edge to true them by. The screws and slots admit also of readjustment of the whole at any time, if by accident or otherwise the parts get displaced or out of true, or if the wooden base should spring by seasoning, &c. Instead of a board as such foundation or support for the several section of hardened straight-edges, a sheet of metal may be used.

To make a hardened straight-edge of six feet in length, I would affix two pieces, three feet each in length, to a six-feet soft metal-plate, and then true them by a four-feet straight-edge. An edge nearer straight and more reliable for one of this length, could be obtained in this way than by making it in a single piece; whilst it also, as in the still longer ones above mentioned, would have the additional advantage of being readily adjustable when out of true. This mode of construction is illustrated in fig. 3.

It is also important for some purposes to have thicker straight-edges than can be conveniently hardened in the manner above described. Such straight-edges are generally made from one-quarter to one-half inch in thickness, and are called by machinists "winders," which name will indicate one of the uses to which they are applied. They must be thick enough to stand firmly upon their edges.

To make a thick straight-edge, therefore, which shall embody the distinguishing characteristic feature of extreme hardness of the edges, in excess of that between the edges, I put two or more hardened straight-edges, of medium thickness, say from an eighth to three-sixteenths of an inch thick, together, by riveting, or any of the known methods of doing such work; and then finish it as one piece, or I attach a thin hardened straight-edge to a thick, unhardened one, or upon any suitable foundation.

It is desirable that thick straight-edges should have one thin edge, and they are generally so constructed so that they can be applied with greater accuracy to the work. To accomplish this in making thick straight-edges, as above described, where two or more pieces are put together, one of the pieces may be wider, and thinner if desirable, than the other or others. In attaching a thin straight-edge to any foundation, as above described, the hardened edge may project beyond the piece to which it is attached, to serve as a thin edge, while the opposite edge of both pieces may be used when it is applied as a "winder."

These graduated and hardened straight-edges, as above described, are of great advantage and utility when clamped together and used as a gauge for gauging wire, &c., or instead of graduating the hardened edges, an unhardened bevelled or plain piece may be graduated and attached to the hardened piece. Such a formed gauge is much used by watchmakers and other mechanics, but they have not heretofore been hardened as above described, and consequently they soon wear out of true. Both plans of constructing this gauge are represented in fig. 5. The side or part A represents it as constructed with a graduated unhardened piece, attached to an ungraduated hardened piece; and the side or part B represents it as constructed with the graduated hardened straight-edge only.

1. I claim a straight-edge, hardened at its edge or edges, and not at its centre, substantially as described.
2. I claim a straight-edge, having a hardened edge or edges, and admitting, when warped by hardening, of being brought into true, substantially as described.
3. I claim a straight-edge, made of two or more thin pieces, having one or both edges hardened, for the purpose of making it thicker, substantially as described.
4. I claim a straight-edge, composed of a thin plate, with hardened edge or edges, and a supporting-bed or plate, substantially as described.
5. I claim a straight-edge, composed of two or more hardened straight-edges, secured end to end, upon a supporting bed-plate.
6. I claim a straight-edge, when constructed as herein set forth, whether the same be used as a single edge or with two opposing edges, as in a gauge, substantially as described.
7. I claim the mode herein described of under-graduating the straight-edges, to compensate for the stretch in hardening.
8. I claim the process herein described of reducing the graduated edges to the proper standard by tempering.

SAMUEL DARLING.

Witnesses:

JOHN E. HALL,  
ALBERT W. PAINÉ.